

## UNITED STATES PATENT OFFICE

2,268,525

## PROCESS OF DRAWING STEEL

Gerhard Roesner, Ludwig Schuster, and Helmuth Ley, Frankfort-on-the-Main, Germany, assignors to American Lurgi Corporation, New York, N. Y., a corporation of New York

No Drawing. Application September 18, 1939,  
Serial No. 295,540. In Germany September 20,  
1938

6 Claims. (Cl. 205—21)

The invention relates to a process of drawing steel, and particularly to the drawing of so-called stainless steel.

The invention involves a novel treating step which precedes the drawing, this step making possible the cold working or cold drawing of high grade steels of austenitic structure, particularly stainless steels containing chromium and/or nickel.

In the past it has been impossible or difficult to subject such steels to cold working and particularly to cold drawing. Such working has therefore required a heating of the steel with an increase in expense and possible injury to the steel itself.

The primary object of the present invention is to provide a treatment which will render the steel capable of being easily cold-worked, and particularly cold-drawn.

In general, the invention includes as its essential step the treatment of the steel with an acid solution containing an easily hydrolyzable ferric salt. While other acids and particularly the known pickling acids may be useful, the halogen acids, and particularly hydrochloric acid, are most satisfactory.

In the preferred form of the invention, use of oxidizing agents in the treating bath is avoided, and preferably a pure hydrochloric acid is used as the acid treating agent.

As addition agents, any easily hydrolyzable ferric salt may be useful. The preferred salt, however, to be used according to the invention is ferric acetate. The proportion of ferric salt should preferably be such that hydrolysis of the ferric salt takes place on the surface of the metal through the consumption of the acid.

The treating step is carried out in the conventional manner usual in pickling, and the material is then capable of being cold-drawn.

Further improvement in ductility can be obtained if the steel is treated with conventional pickling agents normally used with high grade or stainless steels before it is subjected to the procedure described above. Use may be made for this step of mixtures of hydrochloric acid and nitric acid; of sulphuric acid and hydrochloric acid; of nitric and hydrofluoric acids; or of nitric, hydrochloric and hydrofluoric acids. It is particularly desirable to utilize in addition to hydrochloric acid and sulphuric acids a substance capable of yielding active oxygen which may thus oxidize the hydrochloric acid. Potassium persulphate is an example of such a substance.

The following example will demonstrate one method of carrying out the invention:

An austenitic steel of the stainless type containing 18% chromium and 8% nickel was treated for five minutes at a temperature of 98° C. with a pickling bath of the following composition:

|                                                        | Parts by volume |
|--------------------------------------------------------|-----------------|
| Water                                                  | 300             |
| H <sub>2</sub> SO <sub>4</sub> (specific gravity 1.84) | 140             |
| HCl (specific gravity 1.19)                            | 160             |
| 10% aqueous solution of potassium persulphate          | 600             |

The pickled steel was then removed from this bath and treated at a temperature of from 90° C. to 95° C. for 20 minutes in an aqueous solution containing the following amounts of active materials per liter:

19 gr. hydrochloric acid  
10 gr. anhydrous ferric acetate

After this treatment the steel was provided with a usual drawing lubricant such as wool fat and then cold-drawn. It was found that cold drawing was possible and was quite simple.

While we have described herein some embodiments of our invention we wish it to be understood that we do not intend to limit ourselves thereby except within the scope of the appended claims.

We claim:

1. A process of cold drawing stainless steel which comprises treating the steel with a solution of hydrochloric acid which contains easily hydrolyzable ferric salts, and then drawing the steel so treated.

2. A process of cold drawing stainless steel which comprises treating the steel with a solution of hydrochloric acid which contains easily hydrolyzable ferric salts, in such concentration that hydrolysis of such salts takes place on the surface of the metal, and then drawing the steel so treated.

3. A process of cold drawing stainless steel which comprises treating the steel with a solution of hydrochloric acid which contains ferric acetate, and then drawing the steel so treated.

4. A process of cold drawing stainless steel which comprises treating the steel with an aqueous solution containing substantially 19 grams of hydrochloric acid and 10 grams of ferric acetate per liter, and then drawing the steel so treated.

5. A process of cold working stainless steel objects which comprises first pickling the steel,

then treating the steel in a solution of hydrochloric acid which contains an easily hydrolyzable ferric salt, and then drawing the steel.

6. A process of cold working stainless steel objects which comprises first pickling the steel in a 5 pickling mixture containing an oxidizing agent capable of releasing free oxygen, then treating

the steel in a solution of hydrochloric acid which contains an easily hydrolyzable ferric salt, and then drawing the steel.

GERHARD ROESNER.  
LUDWIG SCHUSTER.  
HELMUTH LEY.